

## UNITED STATES PATENT OFFICE

2,194,478

## EXTREME PRESSURE LUBRICANT

Franz Rudolf Moser and Dirk Roelof Nijk,  
 Amsterdam, Netherlands, assignors to Shell  
 Development Company, San Francisco, Calif.,  
 a corporation of Delaware

No Drawing. Application August 2, 1937, Serial  
 No. 156,958. In the Netherlands August 29,  
 1936

11 Claims. (Cl. 87—9)

This invention relates to lubricants suitable for lubrication under very high pressures and at elevated temperatures.

It has already been proposed to add to lubricating oils and greases substances known as extreme pressure substances, which prevent seizure and scoring of metals which are in motion relative to each other under very high pressures. Most of the substances heretofore suggested contain halogen, sulfur or phosphorus in a form conducive to corrosion. The thought generally prevailed that these elements give rise to a chemical reaction to form products which keep the metals separated when the oil film gives way under excessive pressures. It was reasoned that since a chemical reaction is essential to the working of an extreme pressure lubricant, a certain amount of corrosion is indispensable for the activity of extreme pressure substances.

It has further been proposed to use oxyhydrocarbons such as fatty acids, cresols, phthalic acid, etc., for the purpose of enhancing the power of extreme pressure substances. However, these oxyhydrocarbons, when used by themselves, have little, if any, effect in the matter of inducing extreme pressure properties in mineral oils.

It is the purpose of this invention to provide extreme pressure lubricants which are free from corrosiveness and which for their effectiveness apparently do not rely, or rely only partially, on a chemical reaction between the metals and the extreme pressure substances.

We have discovered that aromatic and hydroaromatic compounds built up of at least two 6-carbon rings, standing in close proximity to each other and containing at least two hydroxyl radicals separated from the rings by not more than 1 carbon atom, i. e., they may be attached directly to the ring as in phenols, or may be part of carbo-hydroxyl groups as in benzoic acid or benzyl alcohol, show good extreme pressure qualities when added to lubricating oils in quantities substantially above 1%.

While the presence of two of the hydroxyl radicals is sufficient to impart to the polycyclic compounds extreme pressure properties, additional hydroxyl radicals improve this property. Thus between two substances of equal molecular structure but differing in the number of attached hydroxyl radicals, those containing the larger number of hydroxyls are in general more active. The relative position of the polar radicals in the molecule seems to have little, if any, influence, provided they are present in their free form and not bound as esters, salts, etc.

The compounds of our invention are non-corrosive towards steel, bronze and various bearing metals and in many instances have positive anti-corrosive properties, particularly so if they possess two or more carboxyl radicals. If, furthermore, the compounds are structurally compact, they are also highly resistant to thermal decomposition at the elevated temperatures normally encountered in the lubrication of internal combustion engines and are therefore especially valuable for use in crankcase lubricants for internal combustion engines.

Due to the fact that our compounds possess two or more hydroxyl or carboxyl radicals they have high boiling temperatures, and most of them are substantially non-volatile. This is of obvious advantage in lubricating oils to be used in internal combustion engines.

The solubility of our compounds in hydrocarbon oils is quite low and therefore they are usually used in the form of suspensions rather than solutions. Suspensions may be prepared in any suitable manner, as by dispersing the compounds in the lubricating oil with the aid of a colloid mill, or by dissolving them in a mutual solvent, etc. Substances having a stabilizing effect on the suspension so produced, such as small quantities of fatty acids of the type of stearic acid, may be added to advantage. Owing to their power to preserve the suspension, such substances have frequently the additional effect of enhancing the extreme pressure properties of our compounds, particularly at elevated temperatures, when the suspensions tend to become unstable.

It has been stated hereinbefore that the two or more 6-carbon rings of our compounds should stand in close proximity to each other. By this we mean that the carbocyclic rings should preferably be separated from each other by a chain or chains of not more than two atoms of an element normally capable of firmly linking 6-carbon rings to produce stable compounds, said element having an atomic number below 17. Thus compounds containing two or more 6-carbon rings which are separated by two or less carbon or nitrogen atoms, or by a single atom of the group consisting of oxygen, sulfur and phosphorus, not forming part of the ring, or which are advantageously linked directly without an intermediate atom as in diphenyl, or by common carbon atoms as in naphthalene, are known to be very stable in the absence of other unstable linkages or radicals. While many compounds are known in which the rings are separated by other elements, having atomic numbers above 16 capable of link-

- ing 6-carbon rings, such as As, Sb, Hg, Pb, etc., we have found that such compounds, although sufficiently stable for many purposes are not sufficiently stable to be of practical use in lubrication, particularly at high temperatures or in the presence of moisture, notwithstanding that all of them exhibit extreme pressure properties, provided they have the necessary hydroxyl radicals; and still other compounds in which the link is formed by elements having atomic numbers below 17, other than those enumerated above, such as Mg, Al, Si, are known to be extremely unstable, some of them igniting in contact with air, and others rapidly hydrolyzing in contact with water.
- Derivatives containing the necessary hydroxyl radicals of diphenylethane, diphenylmethane, triphenylmethane, diphenyl, naphthalene, tetraline, anthracene, phenanthrene, picene, chrysene, acridine, phenacine, diphenyloxide, dinaphthyl-oxide, diphenylsulfide, dinaphthylsulfide, carbazol, azobenzol, triphenylphosphine, or homologues of these compounds are examples of suitable compounds.
- In addition, the rings may contain short aliphatic side chains, relatively long side chains of more than 2 carbon atoms being very undesirable as they greatly lower the thermal stability of our compounds.
- The presence of polar radicals other than hydroxyl of the type described in our compounds may be permissible but is usually of little advantage and in many instances of decided disadvantage. For instance amino radicals frequently reduce the resistance of our compounds toward oxidation, halogens tend to make them corrosive, nitro radicals lower the thermal stability, etc.
- The quantity of our compounds required to impart to mineral lubricating oils high pressure resisting properties normally varies between about 1 to 10%.

In the following examples, which illustrate our invention, results are shown of tests, made in the Boerlage Four-ball apparatus described in Engineering, July 14, 1933, with a straight mineral lubricating oil and blends thereof with various compounds of the group herein described.

#### Example I

- 50 A 4% suspension of a methylene dibetanaphthol in a Venezuelan brightstock gave a welding pressure of 300 kg., whereas the unblended oil permitted welding at 150 kg.

#### Example II

- 55 A suspension of 4% of a 1 hydroxy naphthoic acid in the oil of Example I likewise gave a welding pressure of 300 kg.

#### Example III

- 60 The family of diphenylmethanederivatives provides a large number of suitable compounds which may be obtained by condensing polyphenols, as hydroquinone, resorcine, pyrocatechin, phloroglucine, pyrogallol; or carboxyl phenols as salicylic acid, cresotic acid, gallic acid, or naphthols, naphthoic acids, hydroxy anthracene, alizarine, etc.; with a lower aldehyde such as formaldehyde or acetaldehyde. Also mixtures of various phenols may be condensed.

For instance, a mixture of 3 parts of resorcine, 1 part of a 40% aqueous solution of formaldehyde and 20 parts of an 8% aqueous hydrochloric acid is allowed to stand for several hours, during which time a precipitate of methylene diresorcine

is formed, which is filtered off and recrystallized from ethyl alcohol. The product obtained consists of microscopic crystals. A 4% suspension thereof in the brightstock of Example I raised the welding pressure to 500 kg. All parts are by weight.

#### Example IV

180 grams of salicylic acid are heated on a steam bath for 40 hours with 90 grams of a 30% aqueous formaldehyde solution and 640 milliliters concentrated hydrochloric acid. The crystalline salicylic acid is slowly converted to a sandy powder containing methylene disalicylic acid, which is washed with water to remove the free hydrochloric acid, dissolved in dilute ammonia, filtered and reprecipitated with dilute sulfuric acid. A 4% suspension of the product in the lubricating oil of Example I gave a welding pressure of 600 kg.

#### Example V

Methylene digallic acid, obtained in a manner similar to the procedure described in Example IV, in a 4% suspension in the lubricating oil of Example I gave a welding pressure of 500 kg.

#### Example VI

Another large class of suitable compounds known as the rosolic acids or aurines, which are derivatives of triphenyl methane, may be obtained by condensing phenols or carboxyl phenols with oxalic acid in the presence of a condensing agent such as sulfuric acid, zinc chloride, etc. A 4% suspension of aurine or pararosolic acid raised the welding pressure in the lubricating oil of Example I to 400 kg.

#### Example VII

Likewise a 4% suspension of aurine tricarboxylic acid prepared from salicylic acid and an oxidant, e. g. nitrous acid, raised the welding pressure to 500 kg.

#### Example VIII

4% resaureine, prepared from resorcine and formic acid, suspended in the lubricating oil of Example I raised the welding pressure to 600 kg.

#### Example IX

A further large group of useful compounds capable of improving the load carrying capacity of the films of lubricating oils to which they are added, comprises the group of azo compounds obtained from diazotized benzidine, in which both amino radicals are diazotized. Many of these compounds are exceedingly stable at the elevated temperatures to which lubricants may be exposed in the normal course of their usage.

Thus, when coupling 1 mol diazotized benzidine with 2 mols phenol under conditions to produce the azo compound, the product so obtained, added to the lubricating oil of Example I in an amount of 4%, raised the welding pressure of the latter to 300 kg.

A 4% suspension of the product of similarly coupling diazotized benzidine with resorcine, had a welding pressure of 600 kg. A similar suspension of a condensation product of 1 mol diazobenzidine with 2 mols salicylic acid had a welding pressure of 500 kg., and a 4% suspension of an azo compound produced from diazobenzidine and dibetanaphthol had a welding pressure of 600+ kg.

Other hydroxy aromatic compounds such as those enumerated in Example III may also be used for coupling with the diazobenzidine, whereby

powerful extreme pressure compounds are produced.

We claim as our invention:

1. A non-halogenated compounded lubricant comprising a mineral lubricating oil and from 1 to 10% of an organic compound possessing at least two isocyclic 6-carbon rings in close proximity to each other and at least two hydroxyl radicals separated from the rings by not more than 1 carbon atom, said compound being stable under the conditions normally encountered in the lubrication of internal combustion engines and free from alkyl radicals of more than two carbon atoms and radicals tending to induce corrosion.
2. A non-halogenated compounded lubricant comprising a mineral lubricating oil and from 1 to 10% of an organic compound possessing at least two isocyclic 6-carbon rings separated from each other by at least 1 link consisting of less than 3 carbon atoms, said compound having at least 2 hydroxyl radicals separated from the rings by not more than 1 carbon atom, being stable at the temperature normally encountered in the lubrication of internal combustion engines and free from alkyl radicals of more than two carbon atoms and radicals tending to induce corrosion.
3. A non-halogenated compounded lubricant comprising a mineral lubricating oil and from 1 to 10% of an organic compound possessing at least two isocyclic 6-carbon rings separated from each other by at least 1 link consisting of less than 3 nitrogen atoms, said compounds having at least 2 hydroxyl radicals separated from the rings by not more than 1 carbon atom, being stable under the conditions normally encountered in the lubrication of internal combustion engines and free from alkyl radicals of more than two carbon atoms and radicals tending to induce corrosion.
4. A non-halogenated compounded lubricant comprising a mineral lubricating oil and from 1 to 10% of an organic compound possessing at least two isocyclic 6-carbon rings directly coupled and at least 2 hydroxyl radicals separated from the rings by not more than 1 carbon atom, being stable under the conditions normally encountered in the lubrication of internal combustion engines and being free from alkyl radicals of more than two carbon atoms and radicals tending to induce corrosion.
5. A non-halogenated compounded lubricant comprising a mineral lubricating oil and from 1 to 10% of an organic compound possessing at least two isocyclic 6-carbon rings in close proximity to each other and at least 2 hydroxyl radicals directly attached to the rings, said compound being stable under the conditions normally encountered in the lubrication of internal combustion engines and free from alkyl radicals of more than two carbon atoms and radicals tending to induce corrosion.
6. A non-halogenated compounded lubricant comprising a mineral lubricating oil and from 1 to 10% of an organic compound possessing at least two isocyclic 6-carbon rings in close proximity to each other and at least 2 carboxyl radicals directly attached to the rings, said compound being stable under the conditions normally encountered in the lubrication of internal combustion engines and free from alkyl radicals of more than two carbon atoms and radicals tending to induce corrosion.
7. A non-halogenated compounded lubricant comprising a mineral lubricating oil and from 1 to 10% resaurine.
8. A non-halogenated compounded lubricant comprising a mineral lubricating oil and from 1 to 10% methylene disalicylic acid.
9. A non-halogenated compounded lubricant comprising a mineral lubricating oil and from 1 to 10% methylene digallic acid.
10. A non-halogenated compounded lubricant comprising a mineral lubricating oil and from 1 to 10% of an organic compound possessing at least two isocyclic 6-carbon rings separated from each other by at least one link consisting of less than 3 atoms having atomic numbers below 17 and capable of firmly linking 6-carbon rings to produce a stable compound, and said compound having at least 2 hydroxyl radicals separated from the rings by not more than one carbon atom, being stable under the conditions normally encountered in the lubrication of internal combustion engines and free from alkyl radicals of more than two carbon atoms and radicals tending to induce corrosion.
11. A non-halogenated compounded lubricant comprising a mineral lubricating oil and from 1 to 10% of an organic compound possessing at least two isocyclic six carbon rings in close proximity to each other, at least one carboxylic group and at least one hydroxy group attached directly to a ring, said compound being stable under the conditions normally encountered in the lubrication of internal combustion engines, and being free from alkyl radicals of more than two carbon atoms and radicals tending to induce corrosion.

FRANZ RUDOLF MOSER. 55  
DIRK ROELOF NIJK.